

Feb. 2, 1960

R. H. BRAUNLICH

2,923,378

GAS SOLID CONTACT

Filed April 5, 1955



Fig. 1



Fig. 2



Fig. 3

2,923,378

**GAS SOLID CONTACT**

Richard H. Braunlich, West Chester, Pa., assignor to  
American Viscose Corporation, Philadelphia, Pa.,  
a corporation of Delaware

Application April 5, 1955, Serial No. 499,321

5 Claims. (Cl. 183—114.2)

This invention relates to an extruded monofilament containing an inert material and, more particularly, to a pellet-like particle or wafer formed by cutting or slicing an extruded monofilament into predetermined lengths.

In accordance with the present invention, I have found that it is possible to extrude through a suitable spinneret or jet a monofilament, preferably of greater than 50 denier, in which a material suitable for use in various types of chemical processing equipment is bound. The vehicle or binder used in the present invention is preferably cellulosic such as viscose but may be any extrudable material such as cellulose acetate or nylon that can be conveniently and economically employed in the process. Such materials may be polymeric, thermosetting or thermoplastic. The present invention will be described primarily as employing a viscose monofilament in which the material which should be inert to the viscose may be in the range of 25-95% on the basis of the cellulose in the viscose. Under other conditions the inert material may comprise from 15-95% by weight of the final product. Such pellets or particles after regeneration are of great utility in adsorption or extraction columns, ion-exchange columns, chromatography and catalyst beds for liquid and gas phase reactions. Any solid which may be pelletized for use in chemical processing equipment can be incorporated in the present invention in accordance with the particular type of apparatus and process for which it is intended. Such a material will be referred to generally as the inert material to distinguish it from the binder or vehicle. It will be understood, however, that this inert material need only be inert to the particular binder employed and the type of regeneration or setting up that may be required under the circumstances. Since the nozzle or spinneret holes would preferably be on the order of one-sixteenth to one-eighth of an inch in diameter or of a shape providing a corresponding area, the inert material may be comparatively large without danger of plugging the spinneret holes. On the other hand, the present invention permits the use of extremely finely ground material where such is desirable since the extruded monofilament can be regenerated with or without acid by means of a hot water bath, a salt bath, an acid bath or hot gas such as air, steam or nitrogen. With hot gas, an aging accelerator may be incorporated in the mixture before extrusion.

A particularly important feature of the present invention resides in the ability to provide a relative porous pellet or disc which in turn permits complete penetration of the fluid in the bed. The pellets are amorphous and will expand like tiny sponges to permit complete diffusion of liquid or gas through the individual pellets. This represents a distinct advance over the conventional pellets supplied for use in chemical apparatus because only surface contact with the pelletized material has been possible. Furthermore, the movement of the conventional pellets tends to permit small particles or fines to break off. These are carried along with the gas or liquid so that further treatment to remove the fines is fre-

quently required. In addition, many useful catalysts cannot be pelletized in the conventional manner but can be incorporated in the pellets of the present invention.

A primary object of the present invention therefore 5 is to provide an improved pellet for use in chemical processing equipment.

A further object of the invention is to provide a porous pellet for use in chemical processing equipment.

A still further object of the invention is to provide an 10 improved porous pellet having a cellulosic binder.

A further object of the invention is to provide a method 15 for producing a uniform particle or pellet which may be packed into a controlled structure having use in catalyst beds and ion-exchange beds.

A further object of the invention is to provide an 20 improved pellet for chemical processing beds in which the fines are completely bound.

A further object of the invention is to provide an 25 improved method for producing accurately a plurality of pellets having identical amounts of non-cellulosic material.

A further object of the invention is to provide a method 30 for producing cellulosically bound monofilaments.

Further objects will be apparent from the specification 25 and drawings in which:

Figure 1 is a diagrammatic showing of the apparatus for forming a large monofilament in accordance with the present invention;

Figure 2 is a diagrammatic perspective showing a cutter 30 for making small wafers or pellets from the monofilament formed as shown in Figure 1;

Figure 3 is a perspective showing on an enlarged scale one of the pellets.

The invention comprises essentially the formation of 35 a relatively large monofilament extruded into a liquid bath to set up a cellulosic vehicle in which a material useful in some chemical process has been injected. The monofilament can be sliced or chopped into small sections of uniform length so that the quantity of the material in each pellet is accurately known. Preferably, 40 the filament can be regenerated without acid and the material carried by the cellulosic binder would be chosen so that it would be inert to the particular regeneration bath employed as well as inert to the viscose. Examples 45 of such materials are absorbent or adsorbent carbon black, catalysts such as  $Fe_2O_3$ ,  $MgO$ ,  $Cr_2O_3$  and aluminum oxides; in fact, any material which is useful in adsorption or extraction columns, ion-exchange columns, chromatography, catalyst beds for liquid or gas phase reactions. 50 The use of the large extrusion orifice permits nearly any solid which is customarily pelletized for use in chemical processing to be bound in the cellulose monofilament and the regeneration bath would be chosen accordingly.

55 Referring now more particularly to the drawings, a monofilament M is formed by extruding a mixture of liquid cellulosic vehicle such as viscose and the desired inert material through a spinneret 5 into the regenerating bath 6. The filament is carried from the bath 6 over a guide 7 whereupon it may be wound up or stored in any desirable manner or after suitable washing may be directly sliced or pelletized. The monofilament M in Figure 2 may be fed into any slicing machine along a guide 8 and through a plate 9. A revolving blade 10 cuts off or slices predetermined lengths of the filament M to form the wafers or pellets P such as shown in Figure 3. The blade 10 is rotated by means of shaft 11 connected to a suitable source of power not shown.

It will be understood that the pellets formed as described above will have uniform distribution of the material carried in the binder. This will be the case even though excessive grinding is not required before extru-

sion through the spinneret or jet 5. Such pellets or wafers can be counted or weighed to obtain an accurate calculation of the amount of material contained in any given number or volume. They are useful in adsorption columns; for example, activated carbon in the pellets can be used to adsorb ammonia from gas streams. In the liquid phase, they may be used to remove organic material dissolved in water and in packed beds for any type of liquid phase extraction. Ion-exchange and chromatography are other fields which find use for such pelletized material. Generally these uses involve packed beds through which various fluids are passed.

A particularly noteworthy field for the products of the present invention are in catalyst beds for both organic and inorganic reactions. These reactions include synthesis, decomposition, hydration, dehydration, reduction, oxidation, hydrogenation, dehydrogenation, chlorination, dechlorination, bromination, fluorination, iodination, nitration, denitration, sulfurization, desulfurization, alkylation, destructive alkylation, condensation, polymerization, isomerization and cyclization.

Particular benefits to be derived in the practice of the present invention include the ease and low cost of forming the large monofilaments and the pellets. Since the porosity of the bed can be accurately controlled by practicing the present invention, it follows that the pressure drop through the beds can also be controlled and thus undesirable high pressure drop can be avoided. Precise quantity of the inert material present in the bed is capable of accurate control. There is no danger that the particles of the catalyst will be carried out with the gas or liquid when the pellets are used in the gas or liquid phase. It will be understood that the cross-sectional shape of the monofilament may take any desired form such as round, flat, square, etc. The term "pellet" 35 used in the specification and claims is intended to include any thickness of the severed portion of the monofilament whether a very thin wafer-like size or up to rods or bars.

Having thus described my invention, I claim:

1. A process of contacting a fluid with a contact agent selected from the class consisting of catalysts, absorbents and adsorbents, said contact agent being uniformly distributed in a packed bed of a contact material through which the fluid is passed, the contact material being in the form of monofilament sections having a cellulosic body, with particles of the contact agent distributed uniformly within and forming an integral part of said monofilament sections.

2. Process of claim 1 wherein the contact agent is carbon black.

3. Process of claim 1 wherein the contact agent is a metal oxide.

4. Process of claim 1 wherein the particles of contact agent comprise 25-95% by weight of the monofilament.

5. A process for removing ammonia from a gas stream by passing said gas stream through a column of contact material containing activated carbon which selectively adsorbs the ammonia, the contact material being in the form of cellulosic monofilament sections having a cellulosic body, with finely divided particles of activated carbon distributed uniformly within and forming an integral part of said monofilament sections.

#### References Cited in the file of this patent

#### UNITED STATES PATENTS

|           |              |               |
|-----------|--------------|---------------|
| 1,414,194 | Levy         | Apr. 25, 1922 |
| 2,052,588 | Dreyfus      | Sept. 1, 1936 |
| 2,066,339 | Dreyfus      | Jan. 5, 1937  |
| 2,090,560 | Ubbelohde    | Aug. 17, 1937 |
| 2,436,201 | Cole         | Feb. 17, 1948 |
| 2,465,163 | Lockwood     | Mar. 22, 1949 |
| 2,537,992 | Gross et al. | Jan. 16, 1951 |

#### FOREIGN PATENTS

|         |               |               |
|---------|---------------|---------------|
| 655,185 | Great Britain | July 11, 1951 |
|---------|---------------|---------------|

#### OTHER REFERENCES

"Adsorption," by C. L. Mantell, McGraw-Hill Book Co., Inc., New York, 1945, first edition, page 12.